

1

2,937,113

## METHOD OF PRODUCING AN ELECTRODE-CARRYING SILICON SEMICONDUCTOR DEVICE

Adolf Herlet and Hubert Patalong, Pretzfeld, Upper Franconia, and Norbert Schink, Erlangen, Germany, assignors to Siemens-Schuckertwerke Aktiengesellschaft, Berlin-Siemensstadt, Germany, a German corporation

No Drawing. Application October 24, 1958  
Serial No. 769,295

Claims priority, application Germany November 8, 1957

7 Claims. (Cl. 148—1.5)

Our invention relates to a method of producing a semiconductor device of silicon in which one or more electrodes are formed by alloying gold with an admixture of 0.2 to 5%, preferably about 1%, antimony into the surface of a monocrystalline silicon body. Such a method is disclosed and claimed in the copending application Serial No. 657,631, filed May 7, 1957, now Patent No. 2,898,528, and assigned to the assignee of the present invention.

Electric semiconductor devices of the type here concerned may be designed, for example, as rectifiers, power transistors, photodiodes or the like electric devices, in which one or more antimony-containing gold electrodes, depending upon the use of the device, are fused and alloyed together with the semiconductor proper. The electrodes of such devices have been observed to possess faulty alloying spots, particularly if the antimony-containing foil of gold used for producing the electrodes was very thin, as is the case for example, in the manufacture of transistors. The occurrence of such alloying faults in p-n junction devices produced by the above-mentioned alloying method has the detrimental result of reducing the inverse voltage to which the p-n junction can be subjected, or the device may completely lose the desired blocking ability. It has been proposed to minimize the occurrence of such faulty alloying spots by using, for the alloying process, a gold-antimony alloy with a trace content of arsenic.

It is an object of our invention to provide a more reliable method of avoiding the formation of faulty alloying spots.

To this end and in accordance with our invention, we produce the electrode or electrodes on the monocrystalline body of silicon by alloying into the surface zone of this body a gold-antimony alloy which contains traces of sulphur.

We have found that a sulphur content between 10<sup>-4</sup>% and 10<sup>-1</sup>% by weight of the gold-antimony alloy produces most favorable results.

For preparing the sulphur-containing alloy of gold and antimony, it is preferable to initially melt the sulphur in a preliminary or first melting process together with the highly pure antimony. The sulphur may be added to the melt of antimony in pure or in compound form, for example, as antimony-sulphide (Sb<sub>2</sub>S<sub>3</sub>). The antimony thus provided with a content of sulphur or antimony-sulphide is then admixed to the gold by means of a second melting process and, if desired, by additional melting processes. During the subsequent melting processes the proportion of gold can be increased in steps. In the final stage the proportionate amounts should be preferably 99% Au and 1% Sb/S.

According to a modified method of the invention, the sulphur is added in pure or compound form, for example as antimony-sulphide, to a quantity of gold in a first

2

melting process. The gold quantity in this first process may be highly pure or it may already contain antimony. The sulphur or sulphur compound is directly admixed to the melt of gold. This is done by first adding the sulphur or sulphur compound to a portion of the total gold quantity, and by thereafter performing one or more additional melting processes by means of which the ultimate composition is attained by admixing the antimony and stepwise increasing the proportion of gold, for example up to the above-mentioned optimum proportion of 99:1. The sulphur-containing gold-antimony alloy produced in this manner can then be rolled down to a foil having a thickness of 0.05 mm. or less. In form of such a foil the electrode metal can be conveniently handled and used for forming an electrode on the silicon crystal in the manner mentioned above.

The sulphur-containing gold-antimony alloy can be additionally provided with a trace content of arsenic in accordance with the disclosure in the copending application Serial No. 711,967, filed January 29, 1958. Such an addition of arsenic, relating to the percentage by weight of the gold-antimony alloy, is preferably kept between 10<sup>-3</sup>% and 10<sup>-1</sup>%. The admixing of the arsenic can be effected in a similar manner as described above with reference to the sulphur.

The alloying process proper can be performed, for example, with the aid of resilient and adjustable pressure devices into which the silicon discs, faced on both sides with the above-described electrode foils and, if desired, covered by carrier plates, are clamped between pressure plates, for example of graphite, and in this condition is subjected to heating at approximately 700 to 800°C for a few minutes. Another method of forming the electrodes by alloying the foil together with the silicon body comprises embedding the semiconductor and foil assembly into a mass of powder, such as graphite powder, compressing the embedded assembly and heating it at the above-mentioned temperature and for a similar period of time, preferably while applying moderate pressure up to about 1 kg./cm.<sup>2</sup> or less, this latter method being more fully disclosed in the copending application Serial No. 637,029, filed January 29, 1957. In this manner, highly-doped n-type conducting zones can be produced in the silicon discs. Between such a zone and the adjacent zone formed by silicon which remained unaffected by the alloying treatment, there exists a p-n junction if the silicon, prior to the alloying process, had p-type conductives, such a p-n junction having the effect of making the device asymmetrically conductive.

The above-mentioned melting processes for doping the gold with the above-mentioned additional substances, as well as the above-described alloy-fusion process and any subsequent melting processes as may be needed for fastening current supply conductors to the electrodes, are preferably performed in an inert atmosphere, particularly if the process requires a temperature above 500°C. Gases suitable as inert atmospheres are, for example, argon, nitrogen, carbon monoxide. An addition of borax is to be avoided.

It will be obvious to those skilled in the art, upon a study of this disclosure, that our invention permits of various modifications and alterations with respect to the individual components and method steps disclosed, and hence can be embodied in equipment other than as particularly described herein, without departing from the essential features of the invention and within the spirit and scope of the claims annexed hereto.

We claim:

1. A method for producing an electrode-carrying semiconductor device in which the semiconductor is composed of silicon, comprising forming at least one electron of

foil thickness on a silicon monocrystal by alloying into said silicon monocrystal a quantity of gold containing from 0.2% to 5% antimony and a trace content of sulphur to form a junction zone larger than 1 mm.<sup>2</sup> in area, said electrode having an area equal to that of said junction zone, whereby faulty alloying spots in said junction zone are minimized.

2. A method according to claim 1, said trace content of sulphur being between 10<sup>-4</sup>% and 10<sup>-1</sup>% by weight of the total gold-antimony alloy.

3. A method for producing an electrode-carrying semiconductor device in which the semiconductor is composed of silicon comprising forming at least one electrode of foil thickness on a silicon monocrystal by alloying into said silicon monocrystal a quantity of gold containing from 0.2% to 5% antimony and between 10<sup>-4</sup>% and 10<sup>-1</sup>% sulphur to form a junction zone between said electrode and said monocrystal, said electrode having an area equal to that of said junction zone, said sulphur-containing gold-antimony alloy being prepared by admixing a material selected from the group consisting of sulphur, Sb<sub>2</sub>S<sub>3</sub> and Sb<sub>2</sub>S<sub>5</sub>, admixing said selected material with highly pure antimony in a first melting step, and admixing the product of said first melting step to gold of high purity in at least one subsequent melting step, whereby faulty alloying spots in said junction zone are minimized.

4. A method for producing an electrode-carrying semiconductor device in which the semiconductor is composed of silicon, comprising admixing, in a first melting step, a quantity of sulphur contained in a material selected from the group consisting of pure sulphur and antimony sulphide, to a portion of gold, gradually increasing the gold content in at least one subsequent melting step to produce a gold alloy containing from 0.2% to 5% antimony by weight and containing sulphur in an amount between 10<sup>-4</sup>% and 10<sup>-1</sup>% by weight, and forming at least one electrode of foil thickness on a silicon monocrystal by alloying into said silicon monocrystal a quantity of said gold alloy to form a junction zone between said electrode and said monocrystal, said electrode having an area

equal to that of said junction zone, whereby faulty alloying spots in said junction zone are minimized.

5. A method for producing an electrode-carrying semiconductor device in which the semiconductor is composed of silicon, comprising forming at least one electrode of foil thickness on a silicon monocrystal by alloying into said silicon monocrystal a quantity of gold alloy containing from 0.2% to 5% antimony by weight, from 10<sup>-4</sup>% to 10<sup>-1</sup>% sulphur by weight, and containing a trace content of arsenic to form a junction zone between said electrode and said monocrystal, said electrode having an area equal to that of said junction zone, whereby faulty alloying spots in said junction zone are minimized.

10 6. A method for producing an electrode-carrying semiconductor device in which the semiconductor is composed of silicon, comprising forming at least one electrode of foil thickness on a silicon monocrystal by alloying into said silicon monocrystal a quantity of gold alloy containing from 0.2% to 5% antimony by weight, from 10<sup>-4</sup>% to 10<sup>-1</sup>% sulphur by weight, and containing a between 10<sup>-3</sup>% to 10<sup>-1</sup>% arsenic by weight to form a junction zone between said electrode and said monocrystal, said electrode having an area equal to that of said junction zone.

15 7. A method for producing an electrode-carrying semiconductor device in which the semiconductor is composed of silicon, comprising forming at least one electrode of foil thickness on a silicon monocrystal by joining together with said monocrystal a gold alloy of foil thickness containing from 0.2% to 5% antimony by weight and from 10<sup>-4</sup>% to 10<sup>-1</sup>% sulphur by weight to form a junction zone between said electrode and said monocrystal, said electrode having an area equal to that of said junction zone, whereby faulty alloying spots 20 in said junction zone are minimized.

#### References Cited in the file of this patent

#### UNITED STATES PATENTS

|           |                 |               |
|-----------|-----------------|---------------|
| 2,702,360 | Geacoletto      | Feb. 15, 1955 |
| 2,705,768 | Kleimack et al. | Apr. 5, 1955  |
| 2,865,794 | Kroger et al.   | Dec. 23, 1958 |